

1

2,781,319

## LUBRICATING COMPOSITIONS

Emmett R. Barnum and Lyman E. Lorenzen, Berkeley, Calif., assignors to Shell Development Company, New York, N. Y., a corporation of Delaware

No Drawing. Application March 22, 1954,  
Serial No. 417,964

5 Claims. (Cl. 252—47.5)

This invention relates to lubricants and more particularly to new and improved lubricating compositions containing ashless polyfunctional additives which possess particularly pour point depressing and viscosity index improving properties.

Many lubricating oils, because of the nature of their source or methods of refining, contain substantial amounts of wax. Lubricating oils of this type are undesirable or unsuitable for many types of operations, particularly under cold operating conditions such as encountered in cold climates. In order to overcome this defect in wax-containing lubricating oils, pour point depressants and viscosity index improvers have been employed. Among the best known additives of this type are polymeric esters of the acrylic acid series and mixtures of said polymeric materials with other types of polymers such as polymerized olefins, including polyisobutylene, polystyrene, polyindene, polyisoprene and the like, as well as other types of polymeric compounds such as polyvinyl and polyallyl compounds.

Although the above-mentioned polymeric materials can effectively reduce the pour point and improve the viscosity index of oils, they are corrosive; they have a tendency to form emulsions under conditions where water, steam, moisture and the like are encountered; and they possess a tendency to break down at elevated temperatures.

It has now been discovered that the above undesirable effects of polymeric pour point depressants on lubricating oil can be overcome by addition to lubricating oil compositions of from 0.01% to 5%, and preferably from about 0.05 to about 2%, of a highly branched oil-soluble organic compound having an essentially saturated linear hydrocarbon chain of from about 25 to 300 and preferably from 50 to 200 carbon atoms and containing attached to essentially one-half of the chain C-atoms and throughout the length thereof (1) a plurality of non-polar hydrocarbyl radicals of from 8 to about 40 carbon atoms each and (2) a plurality of substituent polar groups



a portion of which may be substituted for by  $R^3X$ —polar groups wherein  $X_1$  and/or  $X_2$  is a chalcogen such as oxygen and/or sulfur,  $R^1$  and  $R^2$  can be the same or different hydrocarbyl radicals, e. g., alkyl, alkaryl, aralkyl, aryl, cycloalkyl radicals or hydrogen at least one of the  $R$ 's being non-aromatic and  $R^3$  can be the same or different from either  $R^1$  or  $R^2$ ; these  $C_8-C_{40}$  hydrocarbyl radicals and polar groups are suitably distributed either uniformly or randomly along the carbon chain, in general being randomly distributed. Preferred polar groups are the



2

and  $R^5O$ —wherein  $R^4$  is a  $C_8-C_{20}$  alkyl (straight or branched) radical and  $R^5$  is the same as  $R^4$  or hydrogen. Other valences of the chain C-atom are satisfied preferably by hydrogen atoms, but may contain some lower alkyl radicals of 1-3 carbons. The ratio of the number of polar groups to the number of non-polar groups can vary within relatively wide limits, e. g., from 1/10 to 5/1 and preferably from 1/3 to 3/1. The compounds or mixtures of such compounds can have a molecular weight or average molecular weight of from about 2,000 to above 100,000 and preferably from 5,000 to 50,000.

Polymeric compounds of this invention can be prepared by hydrolyzing alpha-olefin-vinyl ester copolymers to form polyols and forming polycarbamates from said polyols by reacting them with organic isocyanate and/or isothiocyanate compounds to form the carbamates and derivatives thereof. Another method of preparing polymers of this invention is to react alpha-olefins with a vinyl N or N,N-hydrocarbyl carbamate or thiocarbamate or thiocarbamate such as vinyl N,N-dibutyl carbamate or vinyl N,N-dibutylthiocarbamate. The vinyl carbamates such as vinyl N,N-dihydrocarbyl dithiocarbamate can be prepared by reacting acetylene with an amine and carbon disulfide under super-atmospheric pressure. Other compounds of this type include vinyl N,N-diethyl dithiocarbamate, vinyl N,N'-butyl phenyl dithiocarbamate, vinyl-N hexyl dithiocarbamate, methylallyl carbamate, allyl carbamate and the like. The alpha-olefins used to form copolymers with the carbamates include  $C_8-C_{40}$  alpha-olefins such as alpha-heptadecene, alpha-octadecene, and the like.

The reaction conditions can be varied widely with respect to temperature time ratio of proportion of the reactants and selection of catalysts. Generally the temperature can vary from below room temperature to above 100° C. for a period of a fraction of an hour to over 48 hours, depending upon the reactants and the ratio of the reactants, and catalyst of which preferred are the organic peroxides such as benzoyl peroxide.

Thus, the polycarbamates as well as the polyol-poly carbamates and their thio derivatives used in compositions of this invention are preparable by reacting polyols produced by the method described in patent application Serial No. 357,374, filed May 25, 1953, now abandoned, with organic isocyanates and/or isothiocyanates. Other methods of producing polyols from which the polycarbamates or polythiocarbamates can be produced are described in U. S. Patents 2,421,971 and 2,467,774 or the polyols can be produced by the method described in U. S. Patent 2,551,643 followed by hydrolyzing the copolymer by the method described in the first two patents. Still another method of preparing the polymers of this invention is by the method described in U. S. Patent 2,466,404 as well as by any other suitable means.

The following example illustrates a suitable method of preparing the intermediate product (alkanepolyols) from which the carbamate derivatives can be produced by treating said alkane polyols with organic isocyanate compound and analogues thereof.

60 Example I.—Hydrolysis product of alpha-octadecene-vinyl acetate copolymer

About 1 mole of vinyl acetate and 1.2 moles of alpha-octadecene were thoroughly mixed, a small amount of benzoyl peroxide was added to the mixture and the resulting mixture placed in a glass bomb from which air was displaced by nitrogen. The bomb was placed in a water bath maintained at around 80° C. for a period of about 24 hours. The product was topped to 170° C. at 2 mm. of Hg pressure to remove unreacted material and low molecular weight reaction products. The

residue by analysis had an ester value of 0.491 gram-equivalent of ester groups per 100 grams of sample.

This product was alcoholized in about 1,800 ml. of methanol to which about 1 gram of metallic sodium was added. The mixture was distilled to remove the methyl acetate and the excess methanol and the product was then dispersed in heptane and topped. The resulting residue product was an alkanepolyol (polyhydric alkanol) having a molecular weight of about 8,000 as determined by light scattering on the acetate. From the molecular weight and the aforesaid number of gram equivalents of ester groups of ester groups per 100 grams of the ester, it can be calculated that for the alkanepolyol there is a ratio of alcoholic hydroxyl groups to hydrocarbyl (hexadecyl) radicals of about 2.2. Furthermore, the average alkanepolyol molecule contains about 50 hydroxyethylene radicals and about 23 octadecylene-1,2 radicals; there is a total of about 73 hydrocarbyl and hydroxyl radicals per molecule. In other words, the molecule is a chain of 146 C-atoms having 50 hydroxyl and 23 hexadecyl radicals attached to 73 different C-atoms of the chain throughout the chain length. Those 73 C-atoms having attached thereto 73 C-atoms being saturated with 2 H-atoms each. The molecule can be represented by the formula



*Example II.—Hydrolysis product of alpha-hexadecene-vinyl acetate copolymer*

This copolymer was prepared in accordance with the method of Example I except that alpha-hexadecene was used. The hydrolyzed copolymer was oil-soluble, had a molecular weight of 6,000 to 8,000, an average ratio of 2 hydroxyethylene units for each hexadecylene-1,2 unit.

Other alkanepolyol products suitable for preparation of polycarbamates include the hydrolyzed (alcoholized) copolymers having molecular weights ranging from 6,000 to 12,000 and obtained from the following copolymers:

Alpha-heptadecene-vinyl acetate  
 Alpha-tetradecene-vinyl acetate  
 Alpha-eicosene-vinyl acetate  
 Alpha-octadecene-vinyl propionate  
 Alpha-octadecene-vinyl butyrate  
 Alpha-octadecene-vinyl benzoate  
 Mixtures of alpha-tetradecene and octadecene-vinyl acetate  
 Cracked wax C<sub>18</sub>-C<sub>14</sub> alpha-olefin mixture-vinyl acetate  
 Alpha-docosene-vinyl acetate

The alkane polyols can be prepared by any desired method such as, for example, as described specifically in Examples I and II.

The alkane polyols are converted to corresponding alkane polycarbamates by reacting a plurality (part or all) of the alcoholic groups with an organic isocyanate of an organic isothiocyanate. These isocyanates and isothiocyanates are suitably alkyl, alkenyl, aralkyl, alkaryl, cycloalkyl isocyanates and isothiocyanates illustrated by methyl, propyl, butyl, octyl, 2-ethylhexyl, lauryl, cetyl, dodecyl, hexadecyl, octadecyl, oleyl, ricinoleyl isocyanates and isothiocyanates; phenyl, chlorophenyl, octyl-phenyl isocyanates and isothiocyanates; phenethyl, naphthyl isocyanates and the like.

The following examples are given as illustrative of suitable compounds and of their preparation:

*Example III.—Poly (octadecylcarbamate) of alkanepolyol of Example I*

About one one-fiftieth of a mol of the alkanepolyol product of Example I was reacted with about one mol of octadecylisocyanate in chlorobenzene for a period of about 10 to 24 hours and at reflux temperature. The reaction mixture was then dispersed in acetone and the

resulting white precipitate which formed was filtered and dried. By analysis it was found that the average ratio of hydroxy units to carbamate units in the product was 1:1 and the chain length of the substance remained the same. Thus, it is representable by the formula



The product was oil-soluble and had good pour point depressing properties.

*Example IV.—Poly(octadecylcarbamate) of alkanepolyol of Example II*

About one-fiftieth of a mol of the hydrolysis product of alpha-hexadecene-vinyl acetate copolymer, Example II, was reacted with about one mol of octadecylisocyanate in chlorobenzene for a period of about 16 to 24 hours and at reflux temperature. The product was dispersed in acetone and the white precipitate formed was filtered and dried. The average ratio of hydroxy units and carbamate units in the molecule was 1:1. The product was oil-soluble and had good pour point depressing properties.

*Example V*

A product was prepared by the method of Example III but in which the mol ratio of the copolymer to the isocyanate was in the ratio of 1 to 2, respectively. The product had good oil solubility and pour point depressing properties.

*Example VI*

A product similar to those described above was prepared by reacting alpha-octadecene with vinyl N,N-diethylthiocarbamate in the mol ratio of 1:1 and in the presence of alpha, alpha'-azodiisobutyronitrile as a polymerization initiator for about 6 hours at 55-80° C. The resulting copolymer had good oil-solubility.

*Example VII*

A copolymer of alpha-octadecene and vinylmono-octyl dithiocarbamate was prepared by the method of Example VI using benzoyl peroxide as the catalysts. The copolymer had also good oil-solubility.

*Example VIII*

A copolymer of alpha-octadecene and vinyl N-dodecyl carbamate was prepared as described in Example VI but in which the mol ratio of the reactants was 1 to 2 respectively. The product had good oil-solubility.

Other products useful in lubricating compositions in accordance with this invention are illustrated by those listed below in which the various alkanepolyol compounds (A) are reacted with various isocyanate compounds, (B) the mol ratio of the (A) polyol to the (B) organic isocyanate can be selected to have various values, such as 1:1, 1:2, 1:4, 1:10, 2:1, 4:1, respectively, said polymeric compound having a high molecular weight and good oil solubility: (A) Hydrolyzed (alcoholized) copolymers of alpha-heptadecene/vinyl acetate, alpha-tetradecene/vinyl acetate, alpha-eicosene/vinyl acetate, alpha-octadecene/vinyl propionate, alpha-octadecene/vinyl butyrate, alpha-octadecene/vinyl benzoate; alpha-octadecene/vinyl thioacetate; (B) propyl isocyanate, butyl isocyanate, dodecyl isocyanate, octadecyl isocyanate, oleyl isocyanate, phenyl isocyanate, p-chlorophenyl isocyanate, naphthyl isocyanate, lauryl thioisocyanate, octyldeciyl thioisocyanate, and mixtures thereof.

The base can be any natural or synthetic material having lubricating properties. Thus, the base may be a hydrocarbon oil obtained from a paraffinic, naphthenic, Mid-Continent or Coastal stock and/or mixtures thereof.

The viscosity of these oils may vary over a wide range

such as from 100 SUS at 100° F. to 100 SUS at 210° F. The hydrocarbon oils may be blended with fixed oils such as castor oil, lard oil and the like and/or with synthetic lubricants such as polymerized olefins, copolymers of alkylene glycols and alkylene oxides, organic esters, e. g., 2-ethyl hexyl sebacate, dioctyl phthalate, trioctyl phosphate; polymeric tetrahydrofuran, polyalkyl silicone polymers, e. g., dimethyl silicone polymer and the like. If desired, the synthetic lubricants may be used as the sole base lubricant or admixed with fixed oils and derivatives thereof. In addition, the base can be gasoline, ethyl fluids, fuel oil, greases, etc.

The improved pour point properties which can be imparted to an undoped mineral oil as determined by ASTM procedure is evident from the data presented below.

Table

[Base: Mineral oil]

| Additive         | Amount, percent | ASTM (D-97-47) pour point, °F. |
|------------------|-----------------|--------------------------------|
| Example III----- | 1               | -5                             |
| Example IV-----  | 1               | -5                             |
| Example V-----   | 1               | -5                             |
| None-----        |                 | +20                            |

Compositions of this invention can be modified by addition thereto of minor amounts (0.01-2%) of blooming agents, corrosion inhibitors, oiliness agents, anti-wear agents, solubilizers and the like. Among such materials can be included high molecular weight polymers, e. g., "Acryloids," wax-naphthalene condensation products, isobutylene polymers, alkylstyrene polymers, organic nitrates such as diisopropylammonium nitrite or dicyclohexylammonium nitrite; organic phosphites, phosphates and phosphonates such as trichloroethyl phosphite, tricresyl phosphate, dilorol phosphate, phosphorus sulfide reaction products such as P<sub>2</sub>S<sub>5</sub>-terpene reaction products, metal organic phosphates, e. g., Zn dimethylcyclohexyl phosphate, organic sulfides, e. g., wax disulfide, ethylene bistolyl sulfide; amine, e. g., octadecylamine and the like. Solubilizers for some of the copolymers of this invention which lack desired oil-solubility include long chain aliphatic alcohols and fatty acids such as stearyl alcohol, oleic acid; partial esters such as sorbitan monoleate and the like.

We claim as our invention:

5 1. An improved mineral lubricating oil composition comprising a major amount of mineral lubricating oil and a minor amount, sufficient to depress the pour point of the oil and to improve its viscosity index, of a reaction product obtained by treating (1) a hydrolyzed copolymer of an  $\alpha$ -hydrocarbon olefin of from 8 to 40 carbon atoms and a vinyl ester of a lower fatty acid of up to 5 carbon atoms with (2) an organic isocyanate, said final reaction product having a plurality of hydroxyl and carbamate radicals and the ratio of the number of polar groups to the non-polar groups per molecule varying from 1:10 to 5:1 respectively.

10 2. A composition of claim 1 wherein the average molecule weight of the reaction product is from about 2000 to about 100,000.

15 3. A composition of claim 1 wherein the vinyl ester is vinyl acetate, the organic isocyanate is selected from the group consisting of alkyl isocyanate and alkylisothiocyanate, and said reaction product has an average molecular weight of from about 2,000 to about 100,000.

20 4. A composition of claim 1 wherein the  $\alpha$ -hydrocarbon olefin is  $\alpha$ -hexadecene, the vinyl ester is vinyl acetate, the organic isocyanate is octadecylisocyanate, and the average molecular weight of said reaction product is from about 2,000 to about 100,000.

25 5. A composition of claim 1 wherein the  $\alpha$ -hydrocarbon olefin is  $\alpha$ -octadecene, the vinyl ester is vinyl acetate, the organic isocyanate is octadecylisocyanate, and the average molecular weight of said reaction product is from about 2,000 to about 100,000.

## References Cited in the file of this patent

## UNITED STATES PATENTS

- 35 2,466,404 Fowler ----- Apr. 5, 1949  
 2,483,194 Gleim ----- Sept. 27, 1949  
 2,660,563 Banes et al. ----- Nov. 24, 1953  
 2,737,496 Catlin ----- Mar. 6, 1956

## OTHER REFERENCES

"A New Class of Polymeric Dispersants for Hydrocarbon Systems," presented at the 125 National Meeting, Amer. Chem. Soc., March 23 to April 1, 1954, page 3 pertinent.